

## UNITED STATES PATENT OFFICE

2,632,347

## LUBRICANT FOR METAL ROLLING MILLS

Lorne W. Spreule and Laurence F. King, Sarnia,  
Ontario, Canada, assignors to Standard Oil  
Development Company, a corporation of Delaware

No Drawing. Application March 30, 1949,  
Serial No. 84,484

3 Claims. (Cl. 80—60)

1

The present invention relates to a lubricant for metal rolling mills, and the like, and has particular reference to an improved lubricant composition suitable for use in an aqueous emulsion at the point of roller contact in tin plate production, and the like.

According to the present invention, the rolling of sheet metal such as steel plate, and the like, as in reversing type rolling mills for example, may be considerably facilitated by the use of a lubricant containing specific ingredients. The power requirements for rolling mill operation may be reduced as much as 25% or more, or conversely, the amount of reduction in the thickness of metal plate obtainable for each pass of the rollers may be increased without increasing the power consumption per pass. By this means, the number of passes required to reduce a sheet of steel, for example, from a thickness of about 100/1000" to 10/1000" may be reduced very substantially.

In the prior art, emulsifiable or "soluble" oils have long been used to lubricate the surface of the sheet metal, and thereby reduce rolling friction as well as to cool the sheet metal and the rollers. An emulsion consisting of water with about 1 to 30% by weight of emulsifiable oil therein is sprayed on the sheets as they enter the rollers. The emulsifiable oil ordinarily is cooled and recirculated for reuse. The water is required because of its high heat capacity whereas oil is essential for surface lubrication.

According to the present invention, by incorporating a widely varying quantity, as little as about 0.1% or as much as about 50% by weight, based on the total oil composition (excluding water), of an oiliness or extreme pressure agent into the oil and at the same time changing its emulsification characteristics so that a relatively unstable emulsion is prepared, the reduction in power requirements or the capacity to obtain a greater reduction in thickness per pass may be accomplished. The quantity of emulsifier required will also vary widely, depending upon the other ingredients as well as upon the type of emulsifier.

While the reasons are not too clear why an unstable emulsion should be superior to a stable emulsion, the following explanation is offered as being plausible. In a stable emulsion, the mineral oil content in which an oiliness or extreme pressure agent may be dissolved, is contained in minute globules surrounded by the emulsifier. Emulsifiers commonly used are certain soaps such as sodium naphthenate or sodi-

2

um or calcium sulfonates which are oil-soluble or at least oil dispersible, and the like. Quantities of these may vary from about 2% to 30% by weight of the total oil composition. Other surface active materials may be used with or in lieu of the soaps or sulfonates, e. g. partial C<sub>12</sub> to C<sub>24</sub> fatty acid esters of polyhydric alcohols, and the like. Smaller quantities of these are suitable.

With a stable emulsion there are few if any free particles of oil present which are not protected by the soap or other emulsifier. Apparently, when the metal being rolled comes in contact with such an emulsion, little, if any, oil is held by or adsorbed to the metal because of the presence on the metal surface of a protecting film of soap, sulfonate, or other emulsifier. As a result, there is no surface chemical reaction which can take place directly between the outer layer of molecules of metal and the oiliness or extreme pressure agent. Thus, if the oil contains an extreme pressure agent, such as a phosphorus compound, the emulsifier prevents the immediate reaction between phosphorus and steel which would occur spontaneously at the high instantaneous temperatures at point of rolling contact. This reaction, when it occurs, forms a surface layer of iron phosphide, for example, which appears to have a much lower resistance to rolling than the iron carbide, or the like, which is commonly present on the surface of a rolled steel plate.

On the other hand, where the emulsion is unstable, the oil separates almost instantaneously from the emulsion as the spray strikes the surface of the metal. At the line of rolling contact, the extreme pressure between the plate being rolled and the roller surface causes an instantaneous rise in temperature with the result that the extreme pressure additive immediately reacts with the surface molecules of the plate and the resulting reacted film, for example, iron phosphide or sulfide, is much more readily deformed with the same expenditure of energy. Oiliness agents likewise may react with the metal to form soaps with the same general result. There is some evidence that the soap forming reaction at the rolling temperature is more effective than the conventional phosphide or sulfide reaction.

Thus, it appears that when an emulsifiable oil containing the oiliness or extreme pressure agent is formulated so as to give an unstable or marginally stable emulsion in water, the oil can be adsorbed by the plate and is effective

immediately to reduce friction under boundary conditions of lubrication.

While the above explanation appears to apply specifically to rolling operations, which reduce the thickness of sheet and plate metals, it appears also to have possible application to other metal working operations such as machining, threading, tapping, etc. The essential requirements, for rolling mill lubrication at least, appear to be that the oil shall contain enough of an effective emulsifier to form a true emulsion but that the quantity shall be insufficient to make a stable emulsion. Since the emulsion is circulated in most commercial practice, there is little difficulty in keeping the oil and water sufficiently agitated to retain the emulsion until it can be sprayed or otherwise applied on to the metal ahead of the line of rolling contact. The following specific examples show experimental compositions which gave various results. They demonstrate the difficulty of predicting the results that might be obtained by varying the quantity and types of load carrying agents in the oil. They point clearly, however, to the beneficial effects of controlled emulsification.

#### EXAMPLE A

##### Formula

| Per cent by weight                                            |       |
|---------------------------------------------------------------|-------|
| Sodium sulfonate concentrate (65% sulfonate, 35% mineral oil) | 20.6  |
| Naphthenic acids                                              | 3.25  |
| Sodium hydroxide                                              | 0.5   |
| Water                                                         | 2.15  |
| Alcohol                                                       | 0.5   |
| Candelilla wax                                                | 0.05  |
| Mineral oil, 40 S. U. S. vis. at 210° F                       | 72.95 |

This composition is an emulsifiable oil which forms a stable emulsion with water. It was used as a standard in comparing subsequent examples for their effectiveness as metal rolling lubricants.

#### EXAMPLE B

| Per cent by weight                                           |       |
|--------------------------------------------------------------|-------|
| Sodium sulfonate concentrate (65% sulfonate 35% mineral oil) | 24.0  |
| Naphthenic acids                                             | 3.25  |
| Sodium hydroxide                                             | 0.5   |
| Water                                                        | 2.15  |
| Alcohol                                                      | 0.5   |
| Candelilla wax                                               | 0.05  |
| Mineral oil, 89 S. U. S. vis. at 210° F                      | 69.55 |

This composition is similarly emulsifiable. It showed no improvement over Example A in the rolling of sheet steel.

#### EXAMPLE C

| Per cent by weight                                            |       |
|---------------------------------------------------------------|-------|
| Sodium sulfonate concentrate (65% sulfonate, 35% mineral oil) | 18.5  |
| Naphthenic acids                                              | 3.0   |
| Sodium hydroxide                                              | 0.5   |
| Water                                                         | 2.0   |
| Alcohol                                                       | 0.5   |
| Candelilla wax                                                | 0.05  |
| Mineral oil, 40 S. U. S. vis. at 210° F                       | 74.55 |
| Elaine oil (oleic acid)                                       | 0.28  |
| Sulfur                                                        | 0.62  |

This example was prepared to determine whether the addition of an extreme pressure agent (sulfurized mineral and elaine oil) would

offer substantial improvement. Results were negative.

#### EXAMPLE D

| Per cent by weight                                            |       |
|---------------------------------------------------------------|-------|
| Sodium sulfonate concentrate (65% sulfonate, 35% mineral oil) | 24.5  |
| Naphthenic acids                                              | 3.25  |
| Sodium hydroxide                                              | 0.5   |
| Water                                                         | 2.85  |
| Alcohol                                                       | 1.0   |
| Candelilla wax                                                | 0.05  |
| Sulfurized sperm oil                                          | 10.0  |
| Mineral oil, 40 S. U. S. vis. at 210° F                       | 57.25 |

Like Example C, this example failed to show improvement over the base oil (Example A), notwithstanding the inclusion of a large amount of extreme pressure additive (10% sulfurized sperm oil). The addition of a load bearing agent per se does not solve the problem.

#### EXAMPLE E

| Per cent by weight                                            |       |
|---------------------------------------------------------------|-------|
| Sodium sulfonate concentrate (65% sulfonate, 35% mineral oil) | 13.7  |
| Naphthenic acids                                              | 2.2   |
| Sodium hydroxide                                              | 0.37  |
| Water                                                         | 0.5   |
| Diethylene glycol                                             | 1.1   |
| Mineral oil 50 S. U. S. vis. at 210° F                        | 56.75 |
| Sperm oil                                                     | 25.0  |

This example was similar to Example A except for sperm oil. The use of a very large quantity of an oiliness agent is not effective. Sperm oil is a very good oiliness agent and was used to replace 25% of the mineral oil, without beneficial results.

#### EXAMPLE F

| Per cent by weight                                            |       |
|---------------------------------------------------------------|-------|
| Sodium sulfonate concentrate (65% sulfonate, 35% mineral oil) | 13.7  |
| Naphthenic acids                                              | 2.2   |
| Sodium hydroxide                                              | 0.37  |
| Water                                                         | 0.5   |
| Diethylene glycol                                             | 1.1   |
| Mineral oil 50 S. U. S. vis. at 210° F                        | 71.75 |
| Tricresyl phosphate                                           | 5.0   |
| Sorbitan trioleate                                            | 5.0   |

Tricresyl phosphate is an excellent oiliness agent for many applications but was ineffective here. The sorbitan trioleate was used in addition to the sodium sulfonate as an emulsifier. For some applications this example is a superior lubricant, but it showed no advantages over Example A as a steel rolling lubricant.

#### EXAMPLE G

| Per cent by weight                               |      |
|--------------------------------------------------|------|
| Oleic acid                                       | 30.0 |
| Alkylene oxide derivative of sorbitan monooleate | 15.0 |
| Triethanolamine                                  | 7.5  |
| Mineral oil 50 S. U. S. vis. at 210° F           | 47.5 |

In this example, the oleic acid was only partly saponified, about half being present as free oleic acid, an excellent oiliness agent. The composition was readily emulsifiable however, because of the large soap content, and showed no substantial improvement over Example A. A very slight improvement was noted. Compare the next example.

## 5

## EXAMPLE H

|                                                  | Per cent by weight |
|--------------------------------------------------|--------------------|
| Oleic acid                                       | 10.0               |
| Alkylene oxide derivative of sorbitan monooleate | 5.0                |
| Triethanolamine                                  | 2.5                |
| Mineral oil, 50 S. U. S. vis. at 210° F          | 82.5               |

In this example, the oleic acid was only partly saponified by the triethanolamine, leaving about half as free oleic acid to serve as an oiliness agent. The quantity of soap was insufficient for complete emulsification and this appears to be the reason that this composition showed very superior results in the rolling of steel sheet. This composition showed 5 cc. separation from 100 cc. of 10% emulsion in water after one-half hour.

## EXAMPLE J

|                                                               | Per cent by weight |
|---------------------------------------------------------------|--------------------|
| Sodium sulfonate concentrate (65% sulfonate, 35% mineral oil) | 14.0               |
| Naphthenic acids                                              | 2.25               |
| Sodium hydroxide                                              | 0.35               |
| Water                                                         | 0.10               |
| Diethylene glycol                                             | 1.1                |
| Sperm oil                                                     | 32.0               |
| Mineral oil, 180 S. U. S. vis. at 210° F                      | 50.2               |

Example J was characterized by a heavy mineral oil base. The quantities of sperm oil, as oiliness agent, and of sodium sulfonate, as emulsifier, were rather high, but the composition formed an unstable emulsion in water, showing 7 cc. separation from 100 cc. of 10% emulsion in water. This product gave 0.001 additional reduction in thickness of rolled steel sheets per pass, as compared with Example A. The composition of Example H performed similarly, demonstrating outstanding improvement in these unstable emulsion products.

The data are summarized in the following table:

Table I

| Example                                                                 | A              | B     | C              | D              | E     | F              | G              | H     | J     |
|-------------------------------------------------------------------------|----------------|-------|----------------|----------------|-------|----------------|----------------|-------|-------|
| 10% Emulsion cc. separation after ½ hour                                | no separation. | 1 cc. | no separation. | no separation. | trace | no separation. | no separation. | 5 cc. | 7 cc. |
| Roll Tests (further reduction in thickness in comparison to Example A): |                |       |                |                |       |                |                |       |       |
| 5:1 Dilution                                                            | Blank          | nil   | nil            | nil            | nil   | nil            | 0.0002         | 0.001 | 0.001 |
| 10:1 Dilution                                                           | do             | nil   | nil            | nil            |       |                |                |       |       |

In summary, it will be noted that in Examples A to G inclusive, which form stable emulsions with water there was little variation and no particular advantage in the substitution of various load carrying agents. Thus, the use of waxes, fatty oils, sulfurized fatty oil, tricresyl phosphate, fatty acids and the like, did not appear to make any particular difference in the reduction in thickness for each pass of a steel sheet between rollers. Various dilutions of oil were used, as much as 10%, and high quantities of fatty oil, for example 25% of sperm oil, showed no significant differences.

However, when the quantity of emulsifier was reduced so that 5 to 7 cc. of oil separated from 100 cc. of a 10% emulsion of the oil in water in one-half hour, as in Examples H and J a considerable improvement in rolling effectiveness was obtained. The reductions of about  $\frac{1}{1000}$  per pass above conventional lubricants which were obtained are considered highly satisfactory. The power savings to be obtained from such lubri-

cants are very significant and may be as much as 25% or more.

In general, the quantity of emulsifying agent to make the unstable or marginal emulsion desired will be between 1 and 30% of the weight of the emulsifiable oil, depending upon the other ingredients. The C<sub>12</sub> to C<sub>24</sub> partial esters of the polyhydric alcohols, such as sorbitan monooleate or mono- or distearate, may be used as emulsion agents in proportions of about 0.5 to about 10% by weight, or the alkali or alkaline earth metal sulfonates which are oil soluble, in somewhat larger proportions. A combination of oil soluble metal sulfonates and polyhydric alcohol esters of the type mentioned appears to be preferable. Other suitable emulsifying agents are soaps such as sodium or alkanolamine oleate such as triethanolamine oleate. Where the partial esters and the sulfonates or soaps are both used, the proportions may vary from about 0 to 30% of soap and 0 to 10% of the esters. The quantities preferred are intermediate of these limits.

Specifically, with oils of the types given in Examples H and J, the emulsifiers are about 15 to 18% soap and about 1 to 1.5% glycol (Example J) or about 7 to 8% of the soap triethanolamine oleate.

The oiliness or extreme pressure agents may be referred to generically as load carrying agents. Either may be used, or a combination thereof. The esters of the acids of phosphorus (phosphates and phosphites) as well as the glyceride esters of fatty acids (the common fatty oils), fatty acids and sulphurized fatty acids, and the like are useful as oiliness agents and various extreme pressure additives such as sulfurized and/or phosphorized fatty oils, fatty acids, aliphatic esters, and the like, and the halogenated hydrocarbons, or combinations thereof may be used, as is well understood by those skilled in the art. Tricresyl phosphate, tributyl phosphate, sperm

oil, and closely related materials are specifically preferred as oiliness agents.

What is claimed is:

1. An emulsifiable oil composition of the following approximate formula:

|                                                              | Per cent by weight |
|--------------------------------------------------------------|--------------------|
| Sodium sulfonate concentrate (65% sulfonate 35% mineral oil) | 14.0               |
| Naphthenic acids                                             | 2.25               |
| Sodium hydroxide                                             | 0.35               |
| Water                                                        | 0.10               |
| Diethylene glycol                                            | 1.1                |
| Sperm oil                                                    | 32.0               |
| Mineral oil, 180 S. U. S. viscosity at 210° F                | 50.2               |

2. The process of lubricating metal rolling operations which comprises applying immediately ahead of the line of rolling contact an aqueous emulsion of a composition containing lubricating oil, a load bearing agent and an emulsifying agent added in an amount sufficient

to form a marginally stable, complete emulsion of said composition in water, said emulsion having an equivalent stability such that at least about 50% of said composition separates after 0.5 hour from a 10% emulsion of the composition in the water said emulsion having the property of breaking substantially as it strikes the metal being rolled.

3. An emulsifiable composition having the approximate formula by weight:

15 to 18% soap comprising a major proportion of oil soluble petroleum sulfonate and a minor proportion of sodium naphthenate,

1 to 1.5% diethylene glycol,

About 0.1% water,

About 32% sperm oil,

Balance, mineral lubricating oil.

5  
10  
15

## REFERENCES CITED

The following references are of record in the file of this patent:

## UNITED STATES PATENTS

| Number    | Name           | Date          |
|-----------|----------------|---------------|
| 2,245,649 | Caprio         | June 17, 1941 |
| 2,342,199 | Hurtt          | Feb. 22, 1944 |
| 2,353,830 | Kaufman et al. | July 18, 1944 |
| 2,432,784 | Miller         | Dec. 16, 1947 |
| 2,470,405 | Leland         | May 17, 1949  |
| 2,470,913 | Bjorksten      | May 24, 1949  |

LORNE W. SPROULE.  
LAURENCE F. KING.